

# UNITED STATES PATENT OFFICE.

PIERRE BIRKENSTOCK, OF L'ARBRESLE, FRANCE.

## METHOD FOR THE MANUFACTURE OF BATTING AND YARN OF RAMIE.

949,643.

Specification of Letters Patent. Patented Feb. 15, 1910.

No Drawing.

Application filed September 23, 1909. Serial No. 519,194.

*To all whom it may concern:*

Be it known that I, PIERRE BIRKENSTOCK, citizen of France, residing at 43 Rue de Bordeaux, L'Arbresle, Rhône, France, have 5 invented new and useful Improvements in Methods for the Manufacture of Batting and Yarn of Ramie, of which the following is a specification.

My invention relates to a method concerning more particularly the chemical treatment and the subsequent operations to which the decorticated ramie fibers are submitted in view of obtaining batting and yarn capable of being substituted for batting and 15 yarn of cotton.

The batting and yarn of ramie obtained according to my invention possess the appearance, softness and elasticity of cotton together with a strength much greater than 20 that of the latter, the batting having also the suppleness, fineness, curliness and all properties of cotton batting while the yarn is 30% more resisting than cotton yarn and costs half the price of the same.

25 My method of treating the decorticated ramie is the following, the numbers cited being only indicated by way of example:

(a) 25 kilograms carbonate of soda are placed into 1,000 liters water, the solution is 30 brought to ebullition and then poured over 100 kgr. raw decorticated ramie which is soaked therein for one hour. The bath is then drawn out and the material washed in cold water.

35 (b) 15 liters caustic soda at 42° Baumé are poured into 980 liters of water, 5 liters of sulforicinate of soda at 50% are added and mixed therewith. The 100 kilogr. of ramie treated as under (a) are then placed 40 into the solution which is caused to boil for ten hours. The bath is then drawn out and the material is washed first in cold water containing 1% sulfuric acid and then in pure cold water. Thereafter the material 45 is dried preferably by means of a centrifugal machine.

(c) The ramie treated as described being dried is cut to the length of the fibers to be obtained and passed to the opening machine. 50 The material does not require any combing so that no waste is produced.

(d) When the material is delivered from the opening machine, it is soaked for two hours into a bath containing 250 liters caustic soda at 42° Baumé in 750 liters cold water, wash- 55 ing the same in water containing 1 liter sul-

water. The soda is regenerated for the following operations: for this purpose the material is washed with water containing one liter sulfuric acid in 100 liters water, the material is then washed in pure cold 60 water and dried.

(e) The material is then brought to the spreading or lap machine, carded and spun in the same manner as for cotton, either with floss silk machines or with cotton machines 65 according to the length of the fibers.

The yarn thereby obtained will be preferably treated in a solution containing 500 grams gray soap in 100 liters water. The above mentioned amounts and proportions 70 may be varied within certain limits without departing from the scope of my invention.

Having now described my invention, what I claim as new and desire to secure by Letters Patent is:

1. A method for obtaining ramie yarn, consisting in treating the raw decorticated ramie in a solution of carbonate of soda in water, and washing the same; boiling said material in a solution of caustic soda in 80 water containing sulforicinate of soda, washing the same in cold water containing sulfuric acid and then in pure cold water, and drying the same; cutting the dried material so obtained to the length desired for the 85 fibers and passing the same to the opening machine; treating the material in a solution of caustic soda, washing it in water containing sulfuric acid, then in cold water, and drying the same; treating the material so 90 obtained in the spreading or lap machine, and carding and spinning the same.

2. A method for obtaining ramie yarn, consisting in soaking 100 kgr. of the raw decorticated ramie for one hour in 1,000 95 liters water containing 25 kgr. carbonate of soda and washing the same in cold water; boiling said material for ten hours in a bath formed of 980 liters water containing 15 liters caustic soda at 42° Baumé and 5 liters 100 sulforicinate of soda, and washing the material first in cold water containing 1% sulfuric acid, then in pure cold water, and drying the same; cutting the dried material so obtained to the length desired for the fibers 105 and passing the same to the opening machine; soaking the material for two hours in a bath containing 250 liters caustic soda at 42° Baumé in 750 liters cold water, wash- 110 ing the same in water containing 1 liter sul-

furic acid in 100 liters water, then in pure cold water, and drying the same; treating the material so obtained in the spreading or lap machine and carding and spinning the same and boiling the yarn obtained in a solution containing 500 grams gray soap in 100 liters water.

In testimony whereof I have signed my name to this specification in the presence of two subscribing witnesses.

PIERRE BIRKENSTOCK.

Witnesses:

LEON PELLITÉ,  
MARIN VACHON.